

# United States Patent [19]

Noé

[11] 3,924,428

[45] Dec. 9, 1975

[54] **METHOD OF AND APPARATUS FOR DESCALING AND LEVELING A METAL STRIP**

[75] Inventor: **Oskar Noé**, Mulheim (Ruhr), Germany

[73] Assignee: **Firma BWG Bergwerk- und Walzwerk-Maschinenbau GmbH**, Duisburg, Germany

[22] Filed: **Oct. 7, 1974**

[21] Appl. No.: **512,604**

[30] **Foreign Application Priority Data**

Oct. 8, 1973 Germany ..... 2350503

[52] **U.S. Cl.** ..... **72/40; 29/81 A; 72/161; 72/205; 72/183; 266/3 P**

[51] **Int. Cl.<sup>2</sup>** ..... **B21B 45/06; B21D 1/04**

[58] **Field of Search** ..... 72/39, 40, 205, 161, 160, 72/183; 266/3 P; 134/15, 16, 122; 29/81 A

[56]

**References Cited**

**UNITED STATES PATENTS**

|           |         |                     |          |
|-----------|---------|---------------------|----------|
| 2,163,504 | 6/1959  | Thomas .....        | 29/81 A  |
| 3,261,191 | 7/1966  | Wasson .....        | 72/161   |
| 3,559,431 | 2/1971  | Noe et al. ....     | 72/8     |
| 3,626,735 | 12/1971 | Lebourg et al. .... | 72/205 X |

*Primary Examiner*—Milton S. Mehr  
*Attorney, Agent, or Firm*—Karl F. Ross; Herbert Dubno

[57]

**ABSTRACT**

A metal strip is passed continuously through three succeeding roller-tensioning devices. Between the upstream and central tensioning device the strip is elongated by between 0.5 and 1.3 percent so as to descale this strip. Between the central tensioning device and the downstream tensioning device the strip is elongated by between 2 and 2.5 percent so as to level the strip and prevent end bowing thereof.

**4 Claims, 3 Drawing Figures**





FIG. 2



FIG. 3



## METHOD OF AND APPARATUS FOR DESCALING AND LEVELING A METAL STRIP

### FIELD OF THE INVENTION

The present invention relates to a method of and an apparatus for descaling and leveling a metal strip. More particularly this invention concerns a roller-leveler through which a metal strip is passed before pickling.

### BACKGROUND OF THE INVENTION

Prior to the pickling of a metal strip, in particular a steel strip, it is necessary to descale the strip. This is done in a so-called roller-leveler which stretches the sheet longitudinally to a limited extent while alternately and reverse bending it so as to remove all of the scale thereon. At the same time the strip is flattened.

Experiments have shown that the amount of elongation necessary to descale the strip adequately does not eliminate lateral bowing, that is a deformation of the strip in its own plane toward one side caused by hot-working of the strip. This lateral bowing occurs at the ends of the strip most often so that it is necessary to cut off these ends before the strip can be further processed, as it is impossible to pass the strip through conventional treatment apparatus when it is bowed in this manner.

It has been suggested that this lateral bowing can be eliminated by stretching the strip longitudinally to a relatively large extent. At this high degree of stretch however the descaling is usually insufficient so that the known systems usually employ a degree of stretch that is a middle ground between the two levels, so that the descaling is usually inadequate while the lateral bowing is also insufficiently suppressed.

### OBJECTS OF THE INVENTION

It is therefore an object of the present invention to provide an improved method of an apparatus treating a metal strip.

Another object is the provision of improved system for descaling and leveling a metal strip.

Yet another object is to provide such an apparatus which in one simple operation both effectively descales the strip and leveling it perfectly, thereby eliminating any lateral bowing at the ends thereof.

### SUMMARY OF THE INVENTION

These objects are attained according to the present invention in a system wherein the strip is passed through a pair of succeeding stretching assemblies. In the upstream assembly the strip is subjected to a relatively low degree of longitudinal elongation, equal to the maximum-descaling stretch (MDS). At the downstream assembly the extent of stretch is considerably greater so as to completely eliminate lateral bowing of the strip. Thus in accordance with the present invention the strip in a single pass is both completely descaled and perfectly leveled, both of these operations being carried out at levels which correspond to the ideal stretch for that operation.

In accordance with the present invention the maximum-descaling stretch in the upstream device is between 0.5 percent and 1.3 percent for removal of scale on the strip.

In accordance with yet another feature of this invention the extent of stretch in the downward stream assembly serving to level the strip is greater than 2 percent, advantageously between 2 and 2.5 percent.

The apparatus according to the present invention comprises three roller tensioners separating two reverse bending devices. The strip is descaled between the extreme upstream and the central roller tensioner and is leveled between the central and the extreme downstream roller tensioner.

### BRIEF DESCRIPTION OF THE DRAWING

The above and other objects, features, and advantages will become more readily apparent from the following, reference being made to the accompanying drawing in which:

FIG. 1 is a side view of the system in accordance to the present invention; and

FIGS. 2 and 3 are diagrams illustrating the principles of operation of the system according to the present invention.

### SPECIFIC DESCRIPTION

As shown in FIG. 1 a steel strip 1 is passed in a direction 8 through three succeeding roller-tensioners 2a, 2b, and 2c each having two respective driven tension rollers 3a, 3b, and 3c. Between the upstream roller assembly 2a and the central roller assembly 2b there is provided a reverse-bending device 4' having three reversing rollers 9' much as described in my U.S. Pat. No. 3,777,532 issued on Dec. 11, 1973. Idler rollers 5 are employed to either side of this reverse bender 4' for proper feeding of the strip 1.

A similar reverse bender 4" having rollers 9" is provided between the central tensioning assembly 2b and the downstream tensioning assembly 2c. After exiting from the downstream assembly 2c the strip 1 is pickled.

It has been found that a maximum amount of g/m<sup>2</sup> of scales is removed as illustrated in FIG. 2 when the upstream assembly 2a and the central assembly 2b are so driven as to elongate the strip 1 by an extent equal to the maximum-descaling stretch (MDS) of between 0.5 percent and 1.3 percent. Thus the drive motors 10a and 10b for the assemblies 2a and 2b are so controlled that they stretch the strip between these assemblies by approximately 0.8 percent.

Similarly as shown in FIG. 3 it has been found that the lateral deflection *h* in mm/m of the strip 1 is reduced greatly when the strip 1 is stretched greater than 2 percent. Between 2 and 2.5 percent has been found advantageous. To this end the drive motor 10c of the assembly 2c is driven at a rate relative to the drive speed of the motor 10b of the assembly 2b to stretch the strip 1 between these two assemblies 2b and 2c by an extent equal to between 2 percent and 3 percent.

Thus the band section 6 between the upstream assembly 2a and second assembly 2b is subjected to a longitudinal tension of approximately 10 tons while the tension on the section 7 between the assembly 2b and the assembly 2c is equal to approximately 20 tons.

The system and apparatus according to the present invention is equally usable with nonferrous metal sheets. It is also possible to provide in the system according to the present invention various metal working machines between the rolling-tensioning assemblies 2a - 2c. Four such assemblies could also be provided as could only two to carry out the present invention.

I claim:

1. A method of treating a metal strip comprising the steps of:  
longitudinally stretching said strip to a relatively small extent between 0.5 and 1.3 percent corre-

sponding to maximum-descaling stretch while reverse bending the strip to remove scale from the strip;  
thereafter longitudinally stretching said strip to a relatively large extent sufficient to level said strip;

and

pickling said strip after leveling same.

2. The method defined in claim 1 wherein said strip is leveled by stretching more than 2 percent.

3. An apparatus for treating a metal strip and comprising:

descaling means for longitudinally stretching said strip to a relatively small extent between 0.5 and 1.3 percent to remove scale therefrom;

reverse bending means for reverse bending said strip simultaneously with the longitudinal stretching thereof by said descaling means;

leveling means downstream from said descaling means for stretching said strip to a relatively large extent sufficient to level said strip; and  
means for pickling said strip downstream of said leveling means.

4. The apparatus defined in claim 3 wherein said descaling means includes an upstream roller-tensioner, said leveling means includes a downstream roller-tensioner, and said apparatus includes a central roller tensioner between said upstream and downstream roller tensioners, an upstream reverse bender being provided between said upstream roller-tensioner and said central roller-tensioner and a downstream reverse bender being provided between said central roller-tensioner and said downstream roller-tensioner, each of said reverse benders including a plurality of succeeding and parallel rollers defining a sinusoidal path for said strip.

\* \* \* \* \*

20

25

30

35

40

45

50

55

60

65